

W. White,

Making Hardware.

No 22,466.

Patented Dec. 28, 1858.

Fig. 3.



Fig. 2.



Fig. 1.



Witnesses:

Stephen DeMars  
Peter C. Cleman

Inventor:

William White

# UNITED STATES PATENT OFFICE.

WM. WHITE, OF NEWARK, NEW JERSEY.

## IMPROVEMENT IN MAKING EDGE-TOOLS.

Specification forming part of Letters Patent No. **22,466**, dated December 28, 1858.

*To all whom it may concern:*

Be it known that I, WILLIAM WHITE, of Newark, in the county of Essex and State of New Jersey, have invented a new and improved mode of making edge-tools and other articles from wrought-iron and steel without the usual process of welding and forging or swaging, as now practiced; and I do hereby declare that the following is a full description thereof, reference being had to the accompanying drawings, and to the letters of reference marked thereon.

Figure 1 is a plan of one side of a mold for an ax, A A being half of the recess for the reception of the melted or liquid metal. C is the core-pin to form the eye of the ax; E E, the gate or sprue or passage-way for the metal; F F, the steady-pins.

Fig. 2 represents the opposite side of the mold, B B being the other half of recess A A, Fig. 1; D D, the core-print to fit the other half of core-pin C, Fig. 1. G G are holes for steady-pins F F, Fig. 1.

Fig. 3 represents an edge view in section of Figs. 1 and 2, showing the two halves closed together, the dotted lines representing the recess A A B B for the reception of metal to form an ax, hammer, or other article.

In Fig. 4, (seen in Fig. 2,) 1 2 3 4 5 6 represent the whole ax in a rough state as taken from the mold, with the gate or sprue attached. The red lines divide or distinguish between the head or eye part of ax and the bit or edge part. Each part can be made separate and distinct from the other by the use of a mold the cavity of which shall be the shape of the part desired.

The nature of my invention consists in pouring from a crucible or other vessel into a mold wrought-iron or steel, or both in combination, while in a melted or liquid state, and thereby forming a whole or a part of an ax, hammer, or other article, the cavity of said mold being the shape or form of the article desired.

To enable others skilled in the art to make and use my invention, I will proceed to describe its operation.

I construct my molds from iron or other material, forming the cavity as near to the shape of the article I wish to make as possible. I then secure the two parts of the mold together with a band, clamp, or other device and place it in a convenient place for the reception of the metal, which I reduce to a liq-

uid state by any known process. I build a furnace of fire-brick three feet and four inches deep, two feet and six inches long, and one foot six inches wide, and attach thereto a pipe by which I convey a blast of wind, either hot or cold air. I then cut my iron or steel into small pieces and place it into a crucible, and place the same into the furnace, which is filled two-thirds full of coal or other fuel, and start my fire, applying blast sufficient to reduce the metal to a melted or liquid state. I then pour the liquid metal into the cavity of the mold, using such core-pins and stops as are necessary to obtain the required shape.

Two qualities of metal can be united in the same article by the following method: I place the mold with the edge part of the ax downward, as in Fig. 3. I now pour into the cavity of the mold a very fine quality of cast-steel until it rises up to or a little above the line H, and then from another crucible I pour a mixture of iron and steel or other metal of inferior quality, with which I fill up the head or eye part of the cavity, being very careful to pour from the second crucible at the same time that I cease pouring from the first, so that the stream may not be broken, which will allow the two kinds of metal to unite at or near the line H, and thus form a solid ax from two qualities of metal or from two different kinds of metal—as iron and steel—with out welding and forging or swaging.

I am aware that ingots of steel and iron are now formed by pouring the melted liquid into molds. I do not claim for the purpose of forming the ingot.

I do not claim the manufacture of iron or steel, nor the remelting of the same, either new or old; but

What I claim as my invention, and desire to secure by Letters Patent of the United States, is—

The use of wrought-iron and steel separately or combined while in a melted or liquid state, for the purpose of forming into shape axes and other articles without the process of forging, welding, or swaging, by the use of a mold the cavity of which is the shape or form of the article desired, as set forth in my specification.

WILLIAM WHITE.

Witnesses:

STEPHEN R. HAINES,  
PETER S. CLEARMAN.